



US006068961A

# United States Patent [19]

Dutoff et al.

[11] Patent Number: 6,068,961

[45] Date of Patent: May 30, 2000

[54] TONER PROCESSES

|           |         |                     |         |
|-----------|---------|---------------------|---------|
| 5,585,215 | 12/1996 | Ong et al. ....     | 430/137 |
| 5,650,255 | 7/1997  | Ng et al. ....      | 430/137 |
| 5,650,256 | 7/1997  | Veregin et al. .... | 430/137 |
| 5,766,818 | 6/1998  | Smith et al. ....   | 430/137 |
| 5,928,419 | 7/1999  | Uemura et al. ....  | 106/493 |

[75] Inventors: **Beverly C. Dutoff**, Mississauga; **Paul F. Smith**, Toronto; **Raymond W. Wong**; **Beng S. Ong**, both of Mississauga, all of Canada

[73] Assignee: **Xerox Corporation**, Stamford, Conn.

[21] Appl. No.: 09/259,450

[22] Filed: Mar. 1, 1999

[51] Int. Cl.<sup>7</sup> ..... G03G 9/097

[51] Int. Cl. .... 605G 5/05

[52] U.S. Cl. .... 430/137, 430/109  
[58] **Field of Search** .... 430/137, 109,  
..... 430/45

*Primary Examiner*—John Goodrow  
*Attorney, Agent, or Firm*—E. O. Palazzo

[57] ABSTRACT

A process for the preparation of toner generated by mixing (1) a colorant dispersion preferably containing a nonionic surfactant, and (2) a latex emulsion, and wherein the latex emulsion preferably contains resin, or polymer and a surfactant, and wherein the colorant nonionic surfactant is of the Formulas (I) or (II), or optionally mixtures thereof

[56] **References Cited**

## U.S. PATENT DOCUMENTS

|           |         |                                 |         |
|-----------|---------|---------------------------------|---------|
| 4,558,108 | 12/1985 | Alexandru et al. ....           | 526/340 |
| 4,797,339 | 1/1989  | Maruyama et al. ....            | 430/109 |
| 4,983,488 | 1/1991  | Tan et al. ....                 | 430/137 |
| 4,996,127 | 2/1991  | Hasegawa et al. ....            | 430/109 |
| 5,278,020 | 1/1994  | Grushkin et al. ....            | 430/137 |
| 5,290,654 | 3/1994  | Sacripante et al. ....          | 430/137 |
| 5,308,734 | 5/1994  | Sacripante et al. ....          | 430/137 |
| 5,344,738 | 9/1994  | Kmiecik-Lawrynowicz et al. .... | 430/137 |
| 5,346,797 | 9/1994  | Kmiecik-Lawrynowicz et al. .... | 430/137 |
| 5,348,832 | 9/1994  | Sacripante et al. ....          | 430/109 |
| 5,364,729 | 11/1994 | Kmiecik-Lawrynowicz et al. .... | 430/137 |
| 5,366,841 | 11/1994 | Patel et al. ....               | 430/137 |
| 5,370,963 | 12/1994 | Patel et al. ....               | 430/137 |
| 5,403,693 | 4/1995  | Patel et al. ....               | 430/137 |
| 5,405,728 | 4/1995  | Hopper et al. ....              | 430/137 |
| 5,418,108 | 5/1995  | Kmiecik-Lawrynowicz et al. .... | 430/137 |
| 5,496,676 | 3/1996  | Croucher et al. ....            | 430/137 |
| 5,501,935 | 3/1996  | Patel et al. ....               | 430/137 |
| 5,527,658 | 6/1996  | Hopper et al. ....              | 430/137 |



wherein  $R^1$  is a hydrophobic aliphatic, or hydrophobic aromatic group;  $R^2$  is selected from the group consisting of hydrogen, alkyl, aryl, alkylaryl, and alkylarylalkyl;  $R^3$  is hydrogen or alkyl; A is a hydrophilic polymer chain, and m represents the number of A segments.

**44 Claims, No Drawings**

## TONER PROCESSES

## COPENDING APPLICATIONS AND PATENTS

Illustrated in U.S. Pat. No. 5,944,650, the disclosure of which is totally incorporated herein by reference, are novel surfactants, that is for example, cleavable or hydrolyzable surfactants of the Formulas (I), (II), or (III), and which surfactants, especially those of Formulas (I), (II), or mixtures thereof may be selected for the processes of the present invention. Also, in U.S. Pat. No. 5,766,818, the disclosure of which is totally incorporated herein by reference, there are illustrated toner processes wherein cleavable or hydrolyzable surfactants are selected.

The appropriate components and processes of the above recited application and patent may be selected for the present invention in embodiments thereof.

## BACKGROUND OF THE INVENTION

The present invention is generally directed to toner processes, and more specifically, to aggregation and coalescence or fusion of latex, colorant like pigment, dye, or mixtures thereof, and additive particles, such as known toner additives like charge additives, waxes, and surface additives of silica, metal oxides, metal salts of fatty acids, mixtures thereof, and the like. In embodiments, the present invention is directed to toner processes which provide toner compositions with, for example, a volume average diameter of from about 1 micron to about 20 microns, and preferably from about 2 microns to about 10 microns, and a narrow particle size distribution of, for example, from about 1.10 to about 1.35 as measured by the Coulter Counter method, without the need to resort to conventional pulverization and classification methods, and wherein washing of the toner permits the latex surfactant selected, which can be hydrolyzable, or cleavable, to thereby convert to a substantially inert form, or wherein the surfactant is converted to a form, which is easily removed from the toner, to provide a suitable toner triboelectrical charge, and wherein the removal of the surfactant selected is avoided and washing may not be needed, or wherein washing can be substantially reduced or eliminated. In important embodiments, the present invention relates to the stabilization of colorants, such as pigments, with cleavable nonionic surfactants, and which surfactants can be readily hydrolyzed by, for example, the addition of base to the surfactant in the pH range of from about 8 to about 13 into, or modified into water soluble components for simple washing thereof and removal from the toner generated. In embodiments, the present invention relates to the selection of colorant dispersions preferably containing cleavable surfactants of the formulas illustrated herein, or mixtures thereof, in emulsion/aggregation/coalescence processes, and wherein in embodiments such surfactants contain a phosphate ester linkage in the main chain. The resulting toners can be selected for known electrophotographic imaging and printing processes, including digital color processes.

The toners generated with the processes of the present invention are especially useful for imaging processes, especially xerographic processes, which preferably possess high, for example from about 92 to about 100 percent, toner transfer efficiency, such as those with a compact machine design without a cleaner or those that are designed to provide high quality colored images with excellent image resolution, acceptable signal-to-noise ratio, and image uniformity. Moreover, with the stabilized colorant dispersions there are preferably permitted after removal of the selected

surfactant high stable toner triboelectrical charges, such as from about 20 to about 50 microcoulombs per gram as determined by the known Faraday Cage method, and which triboelectrical values are not substantially adversely effected at a relative humidity of from about 20 to about 80 percent.

## PRIOR ART

There is illustrated in U.S. Pat. No. 4,996,127 a toner of associated particles of secondary particles comprising primary particles of a polymer having acidic or basic polar groups and a coloring agent. The polymers selected for the toners of the '127 patent can be prepared by an emulsion polymerization method, see for example columns 4 and 5 of this patent. In column 7 of this '127 patent, it is indicated that the toner can be prepared by mixing the required amount of coloring agent and optional charge additive with an emulsion of the polymer having an acidic or basic polar group obtained by emulsion polymerization. In U.S. Pat. No. 4,983,488, there is disclosed a process for the preparation of toners by the polymerization of a polymerizable monomer dispersed by emulsification in the presence of a colorant and/or a magnetic powder to prepare a principal resin component and then effecting coagulation of the resulting polymerization liquid in such a manner that the particles in the liquid after coagulation have diameters suitable for a toner. It is indicated in column 9 of this patent that coagulated particles of 1 to 100, and particularly 3 to 70, are obtained. This process results in it is believed in the formation of particles with a wide particle size distribution. The disadvantages of, for example poor particle size distributions usually requiring classification and thus resulting in low toner yields, are illustrated in other prior art, such as U.S. Pat. No. 4,797,339, wherein there is disclosed a process for the preparation of toners by resin emulsion polymerization, wherein similar to the '127 patent certain polar resins are selected; and U.S. Pat. No. 4,558,108, wherein there is disclosed a process for the preparation of a copolymer of styrene and butadiene by specific suspension polymerization. Other prior art that may be of interest includes U.S. Pat. Nos. 3,674,736; 4,137,188 and 5,066,560.

Emulsion/aggregation/coalescence processes for the preparation of toners are illustrated in a number of Xerox patents, the disclosures of each of which are totally incorporated herein by reference, such as U.S. Pat. No. 5,290,654, U.S. Pat. No. 5,278,020, U.S. Pat. No. 5,308,734, U.S. Pat. No. 5,370,963, U.S. Pat. No. 5,344,738, U.S. Pat. No. 5,403,693, U.S. Pat. No. 5,418,108, U.S. Pat. No. 5,364,729, and U.S. Pat. No. 5,346,797; and also of interest may be U.S. Pat. Nos. 5,348,832; 5,405,728; 5,366,841; 5,496,676; 5,527,658; 5,585,215; 5,650,255; 5,650,256 and 5,501,935.

The appropriate components and processes of the above Xerox patents can be selected for the processes of the present invention in embodiments thereof.

## SUMMARY OF THE INVENTION

It is a feature of the present invention to provide toner processes with many of the advantages illustrated herein.

In another feature of the present invention there are provided simple and economical processes for the preparation of black and colored toner compositions with excellent colorant dispersions, thus enabling the achievement of excellent color print quality.

In a further feature of the present invention there is provided a process for the preparation of toner compositions with a volume average diameter of from between about 1 to about 15 microns, and preferably from about 2 to about 10

microns, and a particle size distribution of about 1.10 to about 1.28, and preferably from about 1.15 to about 1.25 as measured by a Coulter Counter without the need to resort to conventional classifications to narrow the toner particle size distribution.

In a further feature of the present invention there is provided a process for the preparation of toner by aggregation and coalescence, or fusion (aggregation/coalescence) of latex, pigment, and additive particles, and wherein there is selected for the pigment dispersion a hydrolyzable nonionic surfactant.

In yet another feature of the present invention there are provided toner compositions with low fusing temperatures of from about 120° C. to about 180° C., and which toner compositions exhibit excellent blocking characteristics at and above about 45° C.

In still a further feature of the present invention there are provided toner compositions which provide high image projection efficiency, such as for example over 75 percent as measured by the Match Scan II spectrophotometer available from Million-Roy.

Aspects of the present invention relate to a process for the preparation of toner comprising mixing (1) a colorant dispersion containing a nonionic surfactant, and (2) a latex emulsion, and wherein the latex emulsion contains resin and a surfactant, and wherein the colorant nonionic surfactant is of the Formulas (I) or (II), or optionally mixtures thereof



wherein  $\text{R}^1$  is a hydrophobic aliphatic, or hydrophobic aromatic group;  $\text{R}^2$  is selected from the group consisting of hydrogen, alkyl, aryl, alkylaryl, and alkylaryalkyl;  $\text{R}^3$  is hydrogen or alkyl;  $\text{A}$  is a hydrophilic polymer chain, and  $m$  represents the number of  $\text{A}$  segments; a process wherein  $\text{R}^1$  is a hydrophobic moiety of alkyl or aryl; and there is accomplished a heating below about or equal to about the resin latex glass transition temperature to form aggregates followed by heating above about or equal to about the resin glass transition temperature to coalesce the aggregates; a process wherein  $\text{R}^1$  is alkyl,  $m$  is a number of from about 2 to about 60, and the hydrophilic polymer  $\text{A}$  is a poly(oxyalkylene glycol) selected from the group consisting of a branched polyoxyalkylene glycol, a block polyoxyalkylene glycol and a homopolymeric polyoxyalkylene glycol; a process wherein  $m$  is a number of from about 5 to about 60, or from about 10 to about 50; a process wherein the weight average molecular weight of  $\text{A}$  is from about 100 to about 3,000; a process wherein  $\text{R}^1$  is methylphenyl, ethylphenyl, propylphenyl, butylphenyl, pentylphenyl, hexylphenyl, octylphenyl, or nonylphenyl;  $\text{R}^2$  is hydrogen, methyl, ethyl, methylphenyl, or propyl;  $\text{R}^3$  is methyl, ethyl, propyl, or butyl; and  $\text{A}$  is polyoxyalkylene glycol, polyethylene glycol, or polypropylene glycol; a process wherein  $\text{R}^1$  is an alkylaryl group, or an alkylaryl group with a substituent of fluoride, chloride, or bromide, wherein alkyl contains from about 2 to about 30 carbon atoms;  $\text{R}^2$  alkyl contains from 1

to about 30 carbon atoms;  $\text{R}^3$  alkyl contains from 1 to about 3 carbon atoms; and wherein  $\text{A}$  is a hydrophilic poly(oxyalkylene glycol) selected from the group consisting of a branched, block or homopolymeric polyoxyalkylene glycol derived from alkylene oxides with from about 2 to about 4 carbon atoms; a process wherein the latex resin is generated from the polymerization of monomers to provide a latex emulsion with submicron resin particles in the size range of from about 0.05 to about 0.3 micron in volume average diameter, and wherein the latex contains an ionic surfactant, a water soluble initiator and a chain transfer agent; adding anionic surfactant to substantially retain the size of the toner aggregates formed; thereafter coalescing or fusing the aggregates by heating; and optionally isolating, washing, and drying the toner; a process wherein isolating, washing and drying are accomplished; a process wherein  $\text{R}^1$  is a an alkylaryl, or an alkylaryl group with a substituent of fluoride, chloride, or bromide, wherein alkyl contains from about 2 to about 30 carbon atoms;  $\text{R}^2$  is an alkyl containing from about 1 to about 30 carbon atoms;  $\text{R}^3$  is a hydrogen or an alkyl of from about 1 to about 3 carbon atoms, wherein  $\text{A}$  is a poly(ethylene glycol); and wherein the molecular weight  $M_w$  of  $\text{A}$  is from about 104 to about 2,500; a process wherein  $\text{R}^2$  is an alkylphenyl with an alkyl of about 4 to about 30 carbon atoms, or wherein  $\text{R}^2$  is an alkyl with from 1 to about 6 carbon atoms; a process wherein the alkylphenyl is an octylphenyl, and  $\text{R}^2$  is a methyl; a process wherein  $\text{R}^2$  is hydrogen or methyl, and wherein the poly(ethylene glycol) has a number of repeat units of from about 4 to about 50; a process wherein the nonionic colorant surfactant is selected in an amount of from about 0.05 to about 60 weight percent based on the total weight of the colorant dispersion solids; a process wherein the surfactant is cleavable, or hydrolyzable, and is selected in an amount of from about 1 to about 12 weight percent; a process wherein the temperature at which the aggregation is accomplished controls the size of the aggregates, and wherein the final toner size is from about 2 to about 15 microns in volume average diameter; a process wherein the aggregation temperature is from about 45° C. to about 55° C., and wherein the coalescence or fusion temperature is from about 85° C. to about 95° C.; a process wherein the colorant is a pigment and wherein the pigment dispersion contains an ionic surfactant, and the latex emulsion contains an ionic surfactant of opposite charge polarity to that of ionic surfactant present in the colorant dispersion; a process wherein the aggregation is accomplished at a temperature of about 15° C. to about 1° C. below the  $T_g$  of the latex resin for a duration of from about 0.5 hour to about 3 hours; and wherein the coalescence or fusion of the components of aggregates for the formation of integral toner particles comprised of colorant, and resin is accomplished at a temperature of from about 85° C. to about 95° C. for a duration of from about 1 hour to about 5 hours; a process wherein the latex resin, or polymer is selected from the group consisting of poly(styrene-alkyl acrylate), poly(styrene-1,3-diene), poly(styrene-alkyl methacrylate), poly(styrene-alkyl acrylate-acrylic acid), poly(styrene-1,3-diene-acrylic acid), poly(styrene-alkyl methacrylate-acrylic acid), poly(alkyl methacrylate-alkyl acrylate), poly(aryl methacrylate-alkyl acrylate), poly(alkyl methacrylate-acrylic acid), poly(styrene-alkyl acrylate-acrylonitrile-acrylic acid), poly(styrene-1,3-diene-acrylonitrile-acrylic acid), and poly(alkyl acrylate-acrylonitrile-acrylic acid); a process wherein the latex resin is selected from the group consisting of poly(styrene-butadiene), poly(methylstyrene-butadiene), poly(methyl methacrylate-butadiene), poly(ethyl methacrylate-

butadiene) poly(propyl methacrylate-butadiene), poly(butyl methacrylate-butadiene), poly(methyl acrylate-butadiene), poly(ethyl acrylate-butadiene), poly(propyl acrylate-butadiene), poly(butyl acrylate-butadiene), poly(styrene-isoprene), poly(methylstyrene-isoprene), poly(methyl methacrylate-isoprene), poly(ethyl methacrylate-isoprene), poly(propyl methacrylate-isoprene), poly(butyl methacrylate-isoprene), poly(methyl acrylate-isoprene), poly(ethyl acrylate-isoprene), poly(propyl acrylate-isoprene), and poly(butyl acrylate-isoprene); poly(styrene-propyl acrylate), poly(styrene-butyl acrylate), poly(styrene-butadiene-acrylic acid), poly(styrene-butadiene-methacrylic acid), poly(styrene-butadiene-acrylonitrile-acrylic acid), poly(styrene-butyl acrylate-acrylic acid), poly(styrene-butyl acrylate-methacrylic acid), poly(styrene-butyl acrylate-acrylonitrile), and poly(styrene-butyl acrylate-acrylonitrile-acrylic acid); and wherein the colorant is a pigment, or a dye; a process wherein the latex surfactant is selected from the group consisting of sodium dodecyl sulfate, sodium dodecylbenzene sulfate and sodium dodecylphthalene sulfate; a process wherein the colorant is carbon black, cyan, yellow, magenta, or mixtures thereof; a process wherein the toner particles isolated are from about 2 to about 10 microns in volume average diameter, and the particle size distribution thereof is from about 1.15 to about 1.30; a process wherein there is added to the surface of the formed toner metal salts, metal salts of fatty acids, silicas, metal oxides, or mixtures thereof, each in an amount of from about 0.1 to about 10 weight percent of the obtained toner particles; a process which comprises mixing a resin latex, an 20 ionic surfactant and the colorant dispersion, and a surfactant of the Formulas (I), or (II); heating the resulting mixture below about, or equal to about the glass transition temperature of the resin; thereafter heating the resulting aggregates above about, or about equal to the glass transition temperature of the resin; and optionally isolating, washing and 25 drying the toner

(I)  
(II)

wherein  $\text{R}^1$  is a hydrophobic group;  $\text{R}^2$  is selected from the group consisting of hydrogen, alkyl, aryl, alkylaryl, and alkylaryalkyl;  $\text{R}^3$  is hydrogen or alkyl;  $\text{A}$  is a hydrophilic segment; and  $m$  represents the number of  $\text{A}$  segments; a process wherein the toner is isolated, washed and dried, and the toner is of a volume average diameter of from about 1 to about 20 microns; a process wherein the colorant nonionic surfactant is selected from the group consisting of poly(ethylene glycol)methyl p-tert-octylphenyl phosphate, poly(ethylene glycol)- $\alpha$ -methyl ether- $\omega$ -methyl p-tert-octylphenyl phosphate, poly(ethylene glycol)methyl decylphenyl phosphate, poly(ethylene glycol)- $\alpha$ -methyl ether- $\omega$ -methyl dodecylphenyl phosphate, poly(ethylene glycol)dodecylphenyl phosphate, bis[poly(ethylene glycol)- $\alpha$ -methyl ether]- $\omega$ -p-tert-octylphenyl phosphate, poly(ethylene glycol)- $\alpha$ , $\omega$ -methyl p-tert-octylphenyl phosphate, poly(ethylene glycol)ethyl p-tert-

octylphenyl phosphate, poly(ethylene glycol)- $\alpha$ -methyl ether- $\omega$ -ethyl p-tert-octylphenyl phosphate, poly(ethylene glycol)phenyl p-tert-octylphenyl phosphate, poly(ethylene glycol)- $\alpha$ -methyl ether- $\omega$ -phenyl p-tert-octylphenyl phosphate, poly(ethylene glycol)tolyl p-tert-octylphenyl phosphate, poly(ethylene glycol)- $\alpha$ -methyl ether- $\omega$ -tolyl p-tert-octylphenyl phosphate, and poly(ethylene oxide-co-propylene oxide)methyl p-tert-octylphenyl phosphate, wherein the polymer chain optionally contains from about 5 to about 50 repeating units or segments process for the preparation of toner comprising mixing a colorant dispersion containing a surfactant with a latex emulsion, and wherein the colorant dispersion surfactant is represented by Formulas 15 (I), (II) or (III); or optionally mixtures thereof



(I)



(II)



(III)

wherein  $\text{R}^1$  is a hydrophobic moiety;  $\text{R}^2$  is selected from the group consisting of hydrogen, alkyl and aryl;  $\text{R}^3$  is hydrogen or alkyl;  $\text{A}$  is a hydrophilic polymer chain; and  $m$  is the number of repeating segments of the hydrophilic polymer chain  $\text{A}$ ; a process wherein the surfactant is nonionic; a process wherein the surfactant is of Formula (I); a process wherein the surfactant is of Formula (II); a process wherein the surfactant is of Formula (III); a process wherein the nonionic surfactant is of Formula (I); a process wherein the nonionic surfactant is of Formula (II); a process wherein the nonionic surfactant is of Formula (III); a process for the stabilization of a colorant dispersion which comprises mixing a colorant and a surfactant represented by Formulas (I), (II) or (III); or optionally mixtures thereof



(I)



(II)

-continued



wherein R<sup>1</sup> is a hydrophobic group; R<sup>2</sup> is hydrogen, aliphatic, or aromatic; A is a hydrophilic chain; and m represent the number of repeating segments; a process wherein the A is polyethylene glycol and the m is a number of about 17; toner emulsion/aggregation/coalescence processes wherein there are selected cleavable nonionic surfactants of the Formulas (I) or (II) illustrated herein, such as poly(ethylene glycol)methyl p-tert-octylphenyl phosphate, wherein the surfactant contains, for example, preferably about 40 ethylene glycol units, poly(ethylene glycol)- $\alpha$ -methyl ether- $\omega$ -methyl p-tert-octylphenyl phosphate wherein the surfactant contains 17 ethylene glycol units or segments, wherein the surfactant is modified or hydrolyzed into a hydrophobic alkylphenol, such as octylphenol, and a hydrophilic polyethylene glycol under basic conditions where the pH is in the range of from about 7 to about 13 and preferably in the range from about 8.5 to about 12; toner processes, especially emulsion/aggregation/coalescence processes wherein there are utilized in such processes non-ionic surfactant compositions of Formulas (I), (II), (III), or mixtures thereof, wherein mixtures can contain for example from about 1 to about 99 weight percent, or parts of the Formula (I) surfactant, and from about 99 to about 1 percent by weight or parts of the surfactant of Formula (II), and which surfactants are comprised of a hydrophobic and a hydrophilic moiety linked together by a phosphate ester linkage, and wherein the nonionic surfactant compositions can be readily decomposed by treatment with a dilute aqueous base solution into water soluble components, which components can be removed from the colorant dispersion generated by washing, thus enabling the provision of toners with excellent charging characteristics; (with the presence of the phosphate ester linkage, the surfactant compositions can, for example, be decomposed, or converted into non-surface-active species or into novel surface-active derivatives with different molecular properties upon exposure to conditions of, for example, basic medium which promote hydrolytic cleavage of the surfactant molecules and toner processes wherein washing substantially removes, or removes the colorant surfactant, and wherein in embodiments the surfactant selected for the colorant dispersion, is a cleavable nonionic surfactant of U.S. Pat. No. 5,944,650, the disclosure of which is totally incorporated herein by reference, and more specifically, is represented by the following Formulas (I) or (II), or mixtures thereof

-continued

(III)

5



wherein R<sup>1</sup> is a hydrophobic aliphatic/aromatic group of, for example, alkyl, aryl, an alkylaryl, or an alkylaryl group with, for example, a suitable substituent, such as halogen like fluorine, chlorine, or bromine, wherein alkyl contains, for example, from about 4 to about 60 carbon atoms and aryl contains from, for example, about 6 to about 60 carbon atoms; R<sup>2</sup> can be selected from the group consisting of hydrogen, alkyl, aryl, alkylaryl, and alkylarylalkyl wherein each alkyl may contain, for example, from 1 to about 6 carbon atoms; R<sup>3</sup> is hydrogen or alkyl of, for example, 1 to about 10 carbon atoms; A is a hydrophilic polymer chain of polyoxyalkylene, polyvinyl alcohols, poly(saccharides), and more specifically, poly(oxalkylene glycols) being selected, for example, from the group consisting of at least one of the heteric, block or homopolymer polyoxyalkylene glycols derived from the same or different alkylene oxides; wherein m is an integer, or a number of from, for example, about 2 to about 500, or about 5 to about 100, and wherein in embodiments the weight average molecular weight, M<sub>w</sub>, of A is, for example, from about 100 to about 300, or from about 104 to about 2,500, and which A is available from Aldrich Chemicals.

In the surfactant, formulas R<sup>1</sup> can be a suitable aliphatic, or a suitable aromatic group, and more specifically R<sup>1</sup> is 30 methylphenyl, ethylphenyl, propylphenyl, butylphenyl, pentylphenyl, hexylphenyl, octylphenyl, or nonylphenyl; R<sup>2</sup> can be hydrogen, a suitable aliphatic, such as alkyl, or aromatic, and more specifically R<sup>2</sup> is methyl, ethyl, methylphenyl, or propyl, R<sup>3</sup> is hydrogen, methyl, ethyl, propyl, or butyl; A can be a glycol, or other similar suitable group, and more specifically R<sup>3</sup> is polyoxyalkylene glycol, polyethylene glycol, or polypropylene glycol, and wherein R<sup>1</sup> is preferably an alkylphenyl such as octylphenyl, R<sup>2</sup> is a methyl, R<sup>3</sup> is methyl and A is polyethylene glycol. The substituents and specific examples thereof are illustrated in copending application U.S. Ser. No. 960,754 (D/97371), the disclosure of which is totally incorporated herein by reference. More specifically, the cleavable nonionic surfactants selected can be of the Formulas (I), (II), or (III), or mixtures thereof, and preferably of Formulas (I) or (II)

(I)



(II)



(III)



(I) 60

65

wherein R<sup>1</sup> is a hydrophobic moiety selected from, for example, the group consisting of alkyl, aryl, and their



substituted derivatives such as those containing a halogen atom such as fluorine, chlorine or bromine, and wherein the alkyl group contains, for example, from about 4 to about 60, and preferably from about 6 to about 30 carbon atoms, and the aryl group contains, for example, from about 6 to about 60, and preferably from about 10 to about 30 carbon atoms; R<sup>2</sup> may be the same as R<sup>1</sup> or different, and can be selected from the group consisting of alkyl, aryl, and their substituted derivatives; R<sup>3</sup> is hydrogen or alkyl of from, for example, about 1 to about 10, and preferably 1 to about 3 carbon atoms; A is a hydrophilic polymer chain selected, for example, from the group consisting of polyoxyalkylene, poly(vinyl alcohols), poly(saccharides) and the like, and preferably is a polyoxyalkylene derived from the same or different alkylene oxides with from about 2 to about 4 carbon atoms; and m is the number of repeating units of the hydrophilic polymer chain, and can be a number of, for example, from about 2 to about 500, and preferably from about 5 to about 100.

Specific examples of surfactants are poly(ethylene glycol) methyl p-tert-octylphenyl phosphate, poly(ethylene glycol)- $\alpha$ -methyl ether- $\omega$ -methyl p-tert-octylphenyl phosphate, poly(ethylene glycol)methyl decylphenyl phosphate, poly(ethylene glycol)- $\alpha$ -methyl ether- $\omega$ -methyl dodecylphenyl phosphate, poly(ethyleneglycol)methyl dodecylphenyl phosphate, bis[poly(ethylene glycol)- $\alpha$ -methyl ether]- $\omega$ -p-tert-octylphenyl phosphate, poly(ethylene glycol)- $\alpha$ , $\omega$ -methyl p-tert-octylphenyl phosphate, poly(ethylene glycol) ethyl p-tert-octylphenyl phosphate, poly(ethylene glycol)- $\alpha$ -methyl ether- $\omega$ -ethyl p-tert-octylphenyl phosphate, poly(ethylene glycol)phenyl p-tert-octylphenyl phosphate, poly(ethylene glycol)- $\alpha$ -methyl ether- $\omega$ -phenyl p-tert-octylphenyl phosphate, poly(ethylene glycol)tolyl p-tert-octylphenyl phosphate, poly(ethylene glycol)- $\alpha$ -methyl ether- $\omega$ -tolyl p-tert-octylphenyl phosphate, and poly(ethylene oxide- $\omega$ -propylene oxide)methyl p-tert-octylphenyl phosphate, and preferably wherein the polymer chain contains from about 5 to about 50 repeating units or segments.

While not being desired to be limited by theory, a possible reaction scheme for the Formula (I) or (II) hydrolysis, or cleaving could be



One important advantage of the processes of the present invention is that the hydrolyzable surfactants can be easily removed from the toner surface and water contamination is avoided, or minimized. Also, removal of the surfactant hydrophilic polyethylene glycol chain from the toner surface prevents adsorption of water by this moiety, and hence enables higher toner triboelectric values under, for example, high humidity conditions.

Embodiments of the present invention include a toner and processes thereof comprising mixing a colorant dispersion and a latex emulsion, and wherein the colorant dispersion contains colorant and a surfactant, and wherein the surfactant is of the Formulas (I) or (II), or optionally mixtures thereof



wherein R<sup>1</sup> is a hydrophobic aliphatic, or hydrophobic aromatic group; R<sup>2</sup> is selected from the group consisting of hydrogen, alkyl, aryl, alkylaryl, and alkylaryalkyl; R<sup>3</sup> is hydrogen or alkyl; A is a hydrophilic polymer chain, and m represents the number of A segments; a process wherein R<sup>1</sup> is a hydrophobic moiety of alkyl or aryl; R<sup>2</sup> is selected from the group consisting of alkyl and aryl; and heating below about or equal to about the resin latex glass transition temperature to form aggregates followed by heating above about or equal to about the resin to coalesce the aggregates; a process wherein R<sup>1</sup> is alkyl, m is a number of from about 2 to about 30, the hydrophilic polymer A is a poly(oxyalkylene glycol) selected from the group consisting of a branched polyoxyalkylene glycol, a block polyoxyalkylene glycol and a homopolymeric polyoxyalkylene glycol; a process wherein m is a number of from about 5 to about 60, or from about 10 to about 30; a process wherein the weight average molecular weight of A is from about 100 to about 4,000; a process wherein R<sup>1</sup> is methylphenyl, ethylphenyl, propylphenyl, butylphenyl, pentylphenyl, hexylphenyl, octylphenyl, or nonylphenyl, R<sup>2</sup> is hydrogen, methyl, ethyl, methylphenyl, or propyl, R<sup>3</sup> is methyl, ethyl, propyl, or butyl, and A is polyoxyalkylene glycol, polyethylene glycol, or polypropylene glycol; a process wherein R<sup>1</sup> is an alkylaryl group, or an alkylaryl group with a substituent of fluorine, chlorine, or bromine, wherein alkyl contains from about 2 to about 34 carbon atoms; R<sup>2</sup> alkyl contains from 1 to about 30 carbon atoms; R<sup>3</sup> alkyl contains from 1 to about 3 carbon atoms; and wherein A is a hydrophilic poly(oxyalkylene glycol) selected from the group consisting of a branched, block or homopolymeric polyoxyalkylene glycol derived from alkylene oxides with from about 2 to about 4 carbon atoms; a process wherein the latex resin is generated from the polymerization of monomers to provide a latex emulsion with submicron resin particles in the size range of from about 0.05 to about 0.3 micron in volume average diameter and wherein the latex contains an ionic surfactant, a water soluble initiator and a chain transfer agent; adding anionic surfactant to retain the size of the toner aggregates formed; thereafter coalescing or fusing the aggregates by heating; and optionally isolating, washing, and drying the toner; a process wherein isolating, washing and drying is accomplished; a process wherein the surfactant is mixed with a basic solution in the pH range of from about 8 to about 13; a process wherein the basic medium, or solution is in the pH range of from about 8.5 to about 12; a process wherein R<sup>1</sup> is an alkylaryl, or an alkylaryl group with a substituent of fluorine, chlorine, or bromine, wherein alkyl contains from about 2 to about 30 carbon atoms; R<sup>2</sup> is an alkyl containing from about 1 to about 30 carbon atoms; R<sup>3</sup> is a hydrogen or an alkyl of from about 1 to about 3 carbon atoms; wherein A is a poly(ethylene glycol); and wherein the molecular weight, M<sub>w</sub>, of A is from about 104 to about 2,500; a process wherein R<sup>2</sup> is an alkylphenyl with an alkyl

of about 4 to about 30 carbon atoms, or wherein R<sup>2</sup> is an alkyl with from 1 to about 6 carbon atoms; a process wherein the alkylphenyl is an octylphenyl, and R<sup>2</sup> is a methyl; a process wherein R<sup>2</sup> is hydrogen or methyl, and wherein the poly(ethylene glycol) has a number of repeat units of from about 4 to about 50; a process wherein the surfactant is selected in an amount of from about 0.05 to about 10 weight percent based on the amount of monomer selected to generate the resin latex; a process wherein the surfactant is cleavable, or hydrolyzable, and is selected in an amount of from about 1 to about 3 weight percent; a process wherein the temperature at which the aggregation is accomplished controls the size of the aggregates, and wherein the final toner size is from about 2 to about 15 microns in volume average diameter; a process wherein the aggregation temperature is from about 45° C. to about 55° C., and wherein the coalescence or fusion temperature is from about 85° C. to about 95° C.; a process wherein the colorant is a pigment and wherein the pigment dispersion contains a nonionic surfactant of Formulas (I) or (II), which surfactant minimizes or prevents water absorption by the toner causing reduced triboelectrical and which surfactant can be easily removed by washing, and the latex emulsion contains an 15 ionic surfactant of opposite charge polarity to that of the nonionic surfactant present in the colorant dispersion; a process wherein the ionic surfactant present in the latex mixture is an anionic surfactant; wherein the aggregation is accomplished at a temperature about 15° C. to about 1° C. below the T<sub>g</sub> of the latex resin for a duration of from about 0.5 hour to about 3 hours; and wherein the coalescence or 20 fusion of the components of aggregates for the formation of integral toner particles comprised of colorant, and resin additives is accomplished at a temperature of from about 85° C. to about 95° C. for a duration of from about 1 hour to about 5 hours; a process wherein the latex resin, or polymer is selected from the group consisting of poly(styrene-alkyl acrylate), poly(styrene-1,3-diene), poly(styrene-alkyl methacrylate), poly(styrene-alkyl acrylate-acrylic acid), poly(styrene-1,3-diene-acrylic acid), poly(styrene-alkyl methacrylate-acrylic acid), poly(alkyl methacrylate-alkyl 25 acrylate), poly(alkyl methacrylate-aryl acrylate), poly(aryl methacrylate-alkyl acrylate), poly(alkyl methacrylate-acrylic acid), poly(styrene-alkyl acrylate-acrylonitrile-acrylic acid), poly(styrene-1,3-diene-acrylonitrile-acrylic acid), and poly(alkyl acrylate-acrylonitrile-acrylic acid), wherein the resin is present in an effective amount of from about 80 percent by weight to about 98 percent by weight of toner, and wherein the colorant is a pigment; a process wherein the latex resin is selected from the group consisting of poly(styrene-butadiene), poly(methylstyrene-butadiene), poly(methyl methacrylate-butadiene), poly(ethyl methacrylate-butadiene), poly(propyl methacrylate-butadiene), poly(butyl methacrylate-butadiene), poly(methyl acrylate-butadiene), poly(ethyl acrylate-butadiene), poly(propyl acrylate-butadiene), poly(butyl acrylate-butadiene), poly(styrene-isoprene), poly(methylstyrene-isoprene), poly(methyl methacrylate-isoprene), poly(ethyl methacrylate-isoprene), poly(propyl methacrylate-isoprene), poly(butyl methacrylate-isoprene), poly(methyl acrylate-isoprene), poly(ethyl acrylate-isoprene), poly(propyl acrylate-isoprene), and poly(butyl acrylate-isoprene); poly(styrene-propyl acrylate), poly(styrene-butyl acrylate), poly(styrene-butadiene-acrylic acid), poly(styrene-butadiene-methacrylic acid), poly(styrene-butadiene-acrylonitrile-acrylic acid), poly(styrene-butyl acrylate-acrylic acid), poly(styrene-butyl acrylate-methacrylic acid), poly(styrene-butyl acrylate- 30 35 40 45 50 55 60 65

acrylonitrile), and poly(styrene-butyl acrylate-acrylonitrile-acrylic acid), and wherein the colorant is a pigment; a process wherein the anionic surfactant is selected from the group consisting of sodium dodecyl sulfate, sodium dodecylbenzene sulfate and sodium dodecylnaphthalene sulfate; a process wherein the colorant is carbon black, cyan, yellow, magenta, or mixtures thereof; a process wherein the toner particles isolated are from about 2 to about 10 microns in volume average diameter, and the particle size distribution thereof is from about 1.15 to about 1.30, wherein the ionic surfactant utilized represents from about 0.01 to about 5 weight percent of the total reaction mixture; a process wherein there is added to the surface of the formed toner metal salts, metal salts of fatty acids, silicas, metal oxides, or mixtures thereof, each in an amount of from about 0.1 to about 10 weight percent of the obtained toner particles; a process which comprises mixing a resin latex, an ionic surfactant and colorant, and wherein the colorant is in the form of a dispersion containing a surfactant of the Formulas (I), or (II); heating the resulting mixture below about, or equal to about the glass transition temperature of the resin; thereafter heating the resulting aggregates above about, or about equal to the glass transition temperature of the resin; and optionally isolating, washing and drying the toner



wherein R<sup>1</sup> is a hydrophobic group; R<sup>2</sup> is selected from the group consisting of hydrogen, alkyl, aryl, alkylaryl, and alkylaryllalkyl; R<sup>3</sup> is hydrogen or alkyl; A is a hydrophilic segment, and m represents the number of A segments; a process wherein the toner is isolated, washed and dried, and the toner is of a volume average diameter of from about 1 to about 20 microns; a process comprising the preparation, or provision of a colorant, especially pigment dispersion containing a cleavable or hydrolyzable nonionic surfactant of the Formulas (I), or (II), and a latex containing a water soluble initiator and a chain transfer agent; aggregating the stabilized colorant dispersion with the latex emulsion and optional additives to form toner sized aggregates; freezing or maintaining the size of aggregates with an anionic surfactant; coalescing or fusing the aggregates by heating; and isolating, washing, and drying the toner



wherein R<sup>1</sup> is alkyl or aryl; R<sup>2</sup> is selected from the group consisting of hydrogen, alkyl and aryl; R<sup>3</sup> is hydrogen or

alkyl; A is a hydrophilic segment, and m represents the number of A segments; a process for the preparation of toner comprising mixing a colorant dispersion with a latex emulsion, and wherein the colorant dispersion contains colorant and a surfactant, and wherein the surfactant is represented by Formulas (I), (II) or (III); or optionally mixtures thereof



wherein  $\text{R}^1$  is a hydrophobic moiety of alkyl or aryl;  $\text{R}^2$  is selected from the group consisting of alkyl and aryl;  $\text{R}^3$  is hydrogen or alkyl; A is a hydrophilic polymer chain; and m is the number of repeating segments of the hydrophilic polymer chain A.

The present invention is, more specifically, directed to a process comprised of blending an aqueous colorant, especially pigment dispersion containing a surfactant of the formulas illustrated herein with a latex emulsion comprised of polymer particles, preferably submicron in size, of from, for example, about 0.05 micron to about 0.1 micron, or from about 0.05 to about 0.5 in volume average diameter, and wherein the nonionic surfactant is, for example, poly (ethylene glycol)methyl p-tert-octylphenyl phosphate, poly (ethylene glycol)- $\alpha$ -methyl ether- $\omega$ -methyl p-tert-octylphenyl phosphate and the like, and an ionic surfactant of opposite charge polarity to that of the nonionic surfactant in the colorant dispersion, thereafter heating the resulting flocculent mixture at, for example, from about 35° C. to about 60° C. (Centigrade) to form toner sized aggregates of from about 2 microns to about 20 microns in volume average diameter, and which toner is comprised of polymer, colorant, such as pigment and optionally additive particles, followed by heating the aggregate suspension at, for example, from about 70° C. to about 100° C. to effect coalescence or fusion of the components of the aggregates and to form mechanically stable integral toner particles.

The particle size of toner compositions provided by the processes of the present invention in embodiments can be controlled by the temperature at which the aggregation of latex, colorant, such as pigment, and optional additives is conducted. In general, the lower the aggregation temperature, the smaller the aggregate size, and thus the final toner size. For a latex polymer with a glass transition temperature (Tg) of about 55° C. and a reaction mixture with a solids content of about 12 percent by weight, an aggregate size of about 7 microns in volume average diameter is obtained at an aggregation temperature of about 53° C.; the same latex will provide an aggregate size of about 5 microns at a temperature of about 48° C. under similar conditions.

Moreover, as illustrated in a related application U.S. Ser. No. 922,437, the disclosure of which is totally incorporated herein by reference, the presence of certain metal ion or metal complexes such as aluminum complex in embodiments enables the coalescence of aggregates to proceed at lower temperature of, for example, less than about 95° C. and with a shorter coalescence time of less than about 5 hours.

In embodiments of the present invention, an aggregate size stabilizer can be added during the coalescence to prevent the aggregates from growing in size with increasing temperature, and which stabilizer is generally an ionic surfactant with a charge polarity opposite to that of the surfactant in the colorant dispersion. In embodiments, the present invention is directed to processes for the preparation of toner compositions which comprises blending an aqueous colorant dispersion preferably containing a pigment, such as carbon black, phthalocyanine, quinacridone or RHODAMINE B™ type, red, green, orange, brown, and the like, with the nonionic surfactant of the formulas illustrated herein, with a latex emulsion derived from the emulsion polymerization of monomers selected, for example, from the group consisting of styrene, butadiene, acrylates, methacrylates, acrylonitrile, acrylic acid, methacrylic acid, and the like, and which latex contains an ionic surfactant such as sodium dodecylbenzene sulfonate, and which latex resin is of a size of, for example, from about 0.05 to about 0.5 micron in volume average diameter; heating the resulting flocculent mixture at a temperature ranging from about 35° C. to about 60° C. for an effective length of time of, for example, 0.5 hour to about 2 hours to form toner sized aggregates; and subsequently heating the aggregate suspension at a temperature at or below about 95° C. to provide toner particles; and finally isolating the toner product by, for example, filtration, washing and drying in an oven, fluid bed dryer, freeze dryer, or spray dryer, and which washing converts the nonionic surfactant into an inert form; whereby surfactant free toner particles comprised of polymer, or resin, colorant, and optional additives are obtained.

Embodiments of the present invention include a process for the preparation of toner comprised of polymer and colorant, especially pigment comprising

- (O) the preparation, or provision of a latex emulsion comprising submicron resin particles, such as styrene, butylacrylate, acrylic acid, which are in the size diameter range of from about 0.05 to about 0.3 microns in volume average diameter in the presence of an ionic surfactant, a water soluble initiator and a chain transfer agent,
- (i) blending an aqueous colorant like a pigment dispersion containing the hydrolyzable nonionic surfactant with the latex emulsion containing an ionic surfactant with a charge polarity opposite to that of the ionic surfactant in the pigment dispersion;
- (ii) heating the resulting mixture at a temperature about 25° C. to about 1° C. below the Tg (glass transition temperature) of the latex polymer to form toner sized aggregates;
- (iii) subsequently stabilizing the aggregates with anionic surfactant and heating the stabilized aggregate suspension to a temperature of about 85° C. to about 95° C. to effect coalescence or fusion of the components of aggregates to enable formation of integral toner particles comprised of polymer, colorant, especially pigment and optional toner additives, such as charge additives; and
- (iv) isolating the toner product by, for example, filtration, followed by washing and drying.

More specifically, the present invention is directed to processes for the preparation of toner compositions by means of a high shearing device, such as a Brinkmann Polytron or IKA homogenizer; (ii) adding the colorant, especially pigment mixture and the cleavable or hydrolyzable nonionic surfactant of the formulas illustrated herein, or mixtures thereof, to a latex emulsion of polymer particles of, for example, poly(styrene-butyl acrylate-acrylic acid), poly(styrene-butadiene-acrylic acid), and the like, an anionic surfactant, such as sodium dodecylsulfate, dodecylbenzene sulfonate or NEOGEN R™, thereby causing a flocculation of pigment, polymer particles and optional additives; (iii) homogenizing the resulting flocculent mixture with a high shearing device, such as a Brinkmann Polytron or IKA homogenizer, and further stirring with a mechanical stirrer at a temperature of about 1° C. to about 25° C. below the Tg of the latex polymer to form toner sized aggregates of from about 2 microns to about 12 microns in volume average diameter; (iv) and heating the mixture in the presence of additional anionic surfactant at a temperature of 95° C. or below for a duration of, for example, from about 1 to about 5 hours to form 2 to 10 micron toner particles with a particle size distribution of from about 1.15 to about 1.35 as measured by the Coulter Counter; and (v) isolating the toner particles by filtration, washing, and drying. Additives to improve flow characteristics and charge additives, if not initially present, to improve charging characteristics may then be added by blending with the formed toner, such additives including AEROSILS® or silicas, metal oxides like tin, titanium and the like, metal salts of fatty acids like zinc stearate, mixtures thereof, and the like, and which additives are present in various effective amounts, such as from about 0.1 to about 10 percent by weight of the toner for each additive.

Illustrative examples of specific latex resin, polymer or polymers selected for the process of the present invention include known polymers such as poly(styrene-butadiene), poly(methyl methacrylate-butadiene), poly(ethyl methacrylate-butadiene), poly(propyl methacrylate-butadiene), poly(butyl methacrylate-butadiene), poly(methyl acrylate-butadiene), poly(ethyl acrylate-butadiene), poly(propyl acrylate-butadiene), poly(butyl acrylate-butadiene), poly(styrene-isoprene), poly(methylstyrene-isoprene), poly(methyl methacrylate-isoprene), poly(ethyl methacrylate-isoprene), poly(propyl methacrylate-isoprene), poly(butyl methacrylate-isoprene), poly(methyl acrylate-isoprene), poly(ethyl acrylate-isoprene), poly(propyl acrylate-isoprene), poly(butyl acrylate-isoprene), poly(styrene-butylacrylate), poly(styrene-butadiene), poly(styrene-isoprene), poly(styrene-butyl methacrylate), poly(styrene-butyl acrylate-acrylic acid), poly(styrene-butadiene-acrylic acid), poly(styrene-isoprene-acrylic acid), poly(styrene-butyl methacrylate-acrylic acid), poly(butyl methacrylate-butyl acrylate), poly(styrene-butyl acrylate-acrylonitrile-acrylic acid), poly(acrylonitrile-butyl acrylate-acrylic acid), and the like. The latex polymer, or resin is generally present in the toner compositions of the present invention in various suitable amounts, such as from about 75 weight percent to about 98, or from about 80 to about 95 weight percent of the toner, and the latex size suitable for the processes of the present invention can be, for example, from about 0.05 micron to about 1 micron in volume average diameter as measured by the Brookhaven nanosize particle analyzer. Other sizes and effective amounts of latex polymer may be selected in embodiments. The total of all toner components, such as resin and colorant, is about 100 percent, or about 100 parts.

The polymer selected for the process of the present invention is preferably prepared by emulsion polymerization methods, and the monomers utilized in such processes include, for example, styrene, acrylates, methacrylates, butadiene, isoprene, acrylic acid, methacrylic acid, acrylonitrile, and the like. Known chain transfer agents, for example dodecanethiol, from, for example, about 0.1 to about 10 percent, or carbon tetrabromide in effective amounts, such as for example from about 0.1 to about 10 percent, can also be utilized to control the molecular weight properties of the polymer when emulsion polymerization is selected. Other processes of obtaining polymer particles of from, for example, about 0.01 micron to about 2 microns can be selected from polymer microsuspension process, such as disclosed in U.S. Pat. No. 3,674,736, the disclosure of which is totally incorporated herein by reference; polymer solution microsuspension process, such as disclosed in U.S. Pat. No. 5,290,654, the disclosure of which is totally incorporated herein by reference, mechanical grinding processes, or other known processes. Also, the reactant initiators, chain transfer agents, and the like as disclosed in U.S. Ser. No. 922,437, now abandoned the disclosure of which is totally incorporated herein by reference, can be selected for the processes of the present invention.

Various known colorants, such as pigments, selected for the processes of the present invention and present in the toner in an effective amount of, for example, from about 1 to about 20 percent by weight of toner, and preferably in an amount of from about 3 to about 10 percent by weight, that can be selected include, for example, carbon black like REGAL 330®; magnetites, such as Mobay magnetites MO8029™, MO8060™; Columbian magnetites; MAPICO BLACKS™ and surface treated magnetites; Pfizer magnetites CB4799™, CB5300™, CB5600™, MCX6369™; Bayer magnetites, BAYFERROX 8600™, 8610™; Northern Pigments magnetites, NP-604™, NP-608™; Magnox magnetites TMB-100™, or TMB-104™; and the like. As colored pigments, there can be selected cyan, magenta, yellow, red, green, brown, blue or mixtures thereof. Specific examples of pigments include phthalocyanine HELIOPHEN BLUE L6900™, D6840™, D7080™, D7020, PYLAM OIL BLUE™, PYLAM OIL YELLOW™, PIGMENT BLUE 1™ available from Paul Uhlich & Company, Inc., PIGMENT VIOLET 1™, PIGMENT RED 48™, LEMON CHROME YELLOW DCC 1026™, E.D. TOLUIDINE RED™ and BON RED C™ available from Dominion Color Corporation, Ltd., Toronto, Ontario, NOVAPERM YELLOW FGL™, HOSTAPERM PINK E™ from Hoechst, and CINQUASIA MAGENTA™ available from E.I. DuPont de Nemours & Company, and the like. Generally, colored pigments that can be selected are cyan, magenta, or yellow pigments, and mixtures thereof. Examples of magentas that may be selected include, for example, 2,9-dimethyl-substituted quinacridone and anthraquinone dye identified in the Color Index as Cl 60710, Cl Dispersed Red 15, diazo dye identified in the Color Index as Cl 26050, Cl Solvent Red 19, and the like. Illustrative examples of cyans that may be selected include copper tetra(octadecyl sulfonamido) phthalocyanine, x-copper phthalocyanine pigment listed in the Color Index as Cl 74160, Cl Pigment Blue, and Anthraquinone Blue, identified in the Color Index as Cl 69810, Special Blue X-2137, and the like; while illustrative examples of yellows that may be selected are diarylide yellow 3,3-dichlorobenzidine acetoacetanilides, a monoazo pigment identified in the Color Index as Cl 12700, Cl Solvent Yellow 16, a nitrophenyl amine sulfonamide identified in the Color Index as Foron Yellow SE/GLN, Cl

Dispersed Yellow 33 2,5-dimethoxy-4-sulfonanilide phenylazo-4'-chloro-2,5-dimethoxy acetoacetanilide, and Permanent Yellow FGL. Colored magnetites, such as mixtures of MAPICO BLACK™, and cyan components may also be selected as pigments with the process of the present invention. Known dyes, such as food dyes and the like, can be selected as the colorant.

Colorants include pigment, dye, mixtures of pigment and dyes, mixtures of pigments, mixtures of dyes, and the like.

Examples of initiators selected for the processes of the present invention include water soluble initiators such as ammonium and potassium persulfates in suitable amounts, such as from about 0.1 to about 8 percent and preferably in the range of from about 0.2 to about 5 percent (weight percent). Examples of organic soluble initiators include Vazo peroxides, such as Vazo 64, 2-methyl 2-2'-azobis propanenitrile, Vazo 88, 2-2'-azobis isobutyramidate dehydrate in a suitable amount, such as in the range of from about 0.1 to about 8 percent. Examples of chain transfer agents include dodecane thiol, octane thiol, carbon tetrabromide and the like in various suitable amounts, such as in the range amount of from about 0.1 to about 10 percent and preferably in the range of from about 0.2 to about 5 percent by weight of monomer.

Surfactants in effective amounts of, for example, from about 0.01 to about 15, or from about 0.01 to about 5 weight percent of the reaction mixture and preferably selected for the latex in embodiments include, for example, anionic surfactants, such as for example, sodium dodecylsulfate (SDS), sodium dodecylbenzene sulfonate, sodium dodecyl-naphthalene sulfate, dialkyl benzenealkyl, sulfates and sulfonates, abitic acid, available from Aldrich, NEOGEN R™, NEOGEN SC™ obtained from Kao, cationic surfactants, such as for example dialkyl benzenealkyl ammonium chloride, lauryl trimethyl ammonium chloride, alkylbenzyl methyl ammonium chloride, alkyl benzyl dimethyl ammonium bromide, benzalkonium chloride, cetyl pyridinium bromide, C12, C<sub>15</sub>, C17 trimethyl ammonium bromides, halide salts of quaternized polyoxyethylalkylamines, dodecylbenzyl triethyl ammonium chloride, MIRAPOL™ and ALKAQUAT™ available from Alkaril Chemical Company, SANIZOL™ (benzalkonium chloride), available from Kao Chemicals, and the like, in effective amounts of, for example, from about 0.01 percent to about 10 percent by weight. Preferably, the molar ratio of the cationic surfactant used for flocculation to the anionic surfactant used in the latex preparation is in the range of from about 0.5 to 4.

Examples of surfactants, which can be added to the aggregates preferably prior to coalescence can be selected from anionic surfactants, such as for example sodium dodecylbenzene sulfonate, sodium dodecylnaphthalene sulfate, dialkyl benzenealkyl, sulfates and sulfonates, abitic acid, available from Aldrich, NEOGEN R™, NEOGEN SC™ obtained from Kao, and the like. They can also be selected from nonionic surfactants such as polyvinyl alcohol, polyacrylic acid, methalose, methyl cellulose, ethyl cellulose, propyl cellulose, hydroxy ethyl cellulose, carboxy methyl cellulose, polyoxyethylene cetyl ether, polyoxyethylene lauryl ether, polyoxyethylene octyl ether, polyoxyethylene octylphenyl ether, polyoxyethylene oleyl ether, polyoxyethylene sorbitan monolaurate, polyoxyethylene stearyl ether, polyoxyethylene nonylphenyl ether, dialkylphenoxy poly(ethyleneoxy) ethanol, available from Rhone-Poulenc as IGEPAL CA-210™, IGEPAL CA-520™, IGEPAL CA-720™, IGEPAL CO-890™, IGEPAL CO-720™, IGEPAL CO-290™, IGEPAL CA-210™, ANTAROX 890™

and ANTAROX 897™, and for the colorant dispersion hydrolyzable or cleavable nonionic surfactants of the formulas illustrated herein, such as poly(ethylene glycol) methyl p-tert-octylphenyl phosphate, wherein the surfactant contains, for example, 40 ethylene glycol units, poly(ethylene glycol)- $\alpha$ -methyl ether- $\omega$ -methyl p-tert-octylphenyl phosphate (wherein the surfactant contains 17 ethylene glycol units). An effective amount of the anionic or nonionic surfactant utilized in the coalescence to stabilize the aggregate size against further growth with temperature is, for example, from about 0.01 to about 10 percent by weight, and preferably from about 0.5 to about 5 percent by weight of reaction mixture.

The toner may also include known charge additives in effective suitable amounts of, for example, from 0.1 to 5 weight percent such as alkyl pyridinium halides, bisulfates, the charge control additives of U.S. Pat. Nos. 3,944,493; 4,007,293; 4,079,014; 4,394,430 and 4,560,635, the disclosures of which are totally incorporated herein by reference, negative charge enhancing additives like aluminum complexes, other known charge additives, and the like.

Surface additives that can be added to the toner compositions after washing or drying include, for example, metal salts, metal salts of fatty acids, colloidal silicas, metal oxides, strontium titanates, mixtures thereof, and the like, which additives are each usually present in an amount of from about 0.1 to about 2 weight percent, reference for example U.S. Pat. Nos. 3,590,000; 3,720,617; 3,655,374 and 3,983,045, the disclosures of which are totally incorporated herein by reference. Preferred additives include zinc stearate and AEROSIL R972® available from Degussa in amounts of from about 0.1 to about 2 percent, which additives can be added during the aggregation or blended into the formed toner product.

Developer compositions can be prepared by mixing the toners obtained with the processes of the present invention with known carrier particles, including coated carriers, such as steel, ferrites, and the like, reference U.S. Pat. Nos. 4,937,166 and 4,935,326, the disclosures of which are totally incorporated herein by reference, for example from about 2 percent toner concentration to about 8 percent toner concentration. The carrier particles can also be comprised of a core with a polymer coating thereover, such as polymethylmethacrylate (PMMA) having dispersed therein a conductive component like conductive carbon black. Carrier coatings include silicone resins, fluoropolymers, mixtures of resins not in close proximity in the triboelectric series, thermosetting resins, and other known components.

Imaging methods are also envisioned with the toners of the present invention, reference for example a number of the patents mentioned herein, and U.S. Pat. Nos. 4,265,660; 4,858,884; 4,584,253 and 4,563,408, the disclosures of which are totally incorporated herein by reference.

The following Examples are being submitted to further define various pieces of the present invention. These Examples are intended to be illustrative only and are not intended to limit the scope of the present invention. Comparative Examples and data are also provided. The surfactants of Formulas (I) or (II) were prepared as illustrated in U.S. Pat. No. 5,944,650, totally incorporated herein by reference.

## EXAMPLE I

### Latex Preparation

A latex emulsion comprised of polymer particles generated from the emulsion polymerization of styrene, butyl acrylate and acrylic acid was prepared as follows. A mixture of 2,255 grams of styrene, 495 grams of butyl acrylate, 55.0

grams of acrylic acid, 27.5 grams of carbon tetrabromide and 96.25 grams of dodecane thiol was added to an aqueous solution prepared from 27.5 grams of ammonium persulfate in 1,000 milliliters of water and 2,500 milliliters of an aqueous solution containing 62 grams of anionic surfactant, NEOGEN R™ and 33 grams of poly(ethylene glycol)- $\alpha$ -methyl ether- $\omega$ -methyl p-tert-octylphenyl phosphate hydrolyzable cleavable nonionic surfactant. The resulting mixture was homogenized at room temperature, about 25° C., under a nitrogen atmosphere for 30 minutes. Subsequently, the mixture was stirred and heated to 70° C. (Centigrade throughout) at a rate of 1° C. per minute, and retained at this temperature for 6 hours. The resulting latex polymer of poly(styrene-co butyl acrylate- $\omega$ -acrylic acid) possessed an  $M_w$  of 24,194, an  $M_n$  of 7,212, measured by Gel Permeation Chromatography, and a mid-point Tg of 57.6° C. measured using Differential Scanning Calorimetry.

#### Preparation of Cyan Pigment Dispersion

##### 5% Solids Loading with 1:1 Ratio of Surfactant to Pigment

12.5 Grams of poly(ethylene glycol)- $\alpha$ -methyl ether- $\omega$ -methyl p-tert-octylphenyl phosphate hydrolyzable cleavable nonionic surfactant, 12.5 grams of Sunfast Blue 15:3 pigment and 475 grams of distilled water, were mixed in a Microfluidizer (Microfluidizer Corporation, Model Number M110-Y), at 15,000 psi for 5 cycles.

To assess stability of the cyan pigment dispersion, two methods were used

- i) The dispersion was centrifuged at 4,000 rpm for 2 minutes and the weight of sediment measured.
- ii) The dispersion was retained, without agitation for 2 months, and the sediment amount measured.

#### Results

The above pigment dispersion showed excellent stability with no sediment measured from either of the above sedimentation methods.

Thus the nonionic surfactant can be applied to pigment dispersions and also the use of the cleavable surfactants in the colorant dispersion can have important implications to the fields of general pigment chemistry.

#### Aggregation of Cyan Toner

260.0 Grams of the latex emulsion as prepared in Example I and 220.0 grams of a dilute aqueous cyan pigment dispersion containing 162 grams of the cyan pigment 15.3 dispersion prepared as above with 2.4 grams of cationic surfactant, SANIZOL B™ and 55.6 grams of deionized water. This dispersion and latex were simultaneously added to 400 milliliters of water with high shear stirring by means of a polytron. The mixture was transferred to a 2 liter reaction vessel and heated at a temperature of 50° C. for 2.0 hours resulting in aggregates of a size of 5.5 micron and a GSD of 1.21 before 30 milliliters of 20 percent aqueous NEOGEN R™ solution was added. Subsequently, the resulting mixture was heated to 95° C. and retained there for a period of 4 hours before cooling down to room temperature, about 25° C. throughout, filtered, washed with water at pH 10, using KOH, and dried in a freeze dryer. The final toner product was comprised of 96.25 percent of the polymer of Example I and 3.75 percent of pigment with a toner particle size of 5.9 microns in volume average diameter and with a particle size distribution of 1.23 both as measured on a Coulter Counter. The morphology was shown to be of a potato shape by scanning electron microscopy. The toner tribo charge following 2 washing steps with water and as determined by the Faraday Cage method throughout was -50 and -26 microcoulombs per gram at 20 and 80 percent relative humidity, respectively, measured on a carrier with a core of a ferrite, about 90 microns in diameter, with a coating

of polymethylmethacrylate and carbon black, about 20 weight percent dispersed therein.

#### Comparative Aggregation of Cyan Toner

260.0 Grams of the latex emulsion as prepared in Example I and 220.0 grams of an aqueous cyan pigment dispersion containing 7.6 grams of cyan pigment 15.3 having a solids loading of 53.4 percent, 2.4 grams of cationic surfactant, SANIZOL B™ were simultaneously added to 400 milliliters of water with high shear stirring by means of a polytron. The mixture was transferred to a 2 liter reaction vessel and heated at a temperature of 50° C. for 2.0 hours resulting in aggregates of a size of 5.9 micron and a GSD of 1.20 before 30 milliliters of 20 percent aqueous NEOGEN R™ solution were added. Subsequently, the resulting mixture was heated to 95° C. and retained there for a period of 4 hours before cooling down to room temperature, about 25° C. throughout, filtered, washed with water at pH 10, using KOH, and dried in a freeze dryer. The final toner product was comprised of 96.25 percent of the polymer of Example I and 3.75 percent of pigment with a toner particle size of 6.1 microns in volume average diameter and with a particle size distribution of 1.20 both as measured on a Coulter Counter. The morphology was shown to be of a potato shape by scanning electron microscopy. The toner tribo charge, following 2 washing steps with water, and as determined by the Faraday Cage method throughout was -44 and -22 microcoulombs per gram at 20 and 80 percent relative humidity, respectively, measured on a carrier with a core of a ferrite, about 90 microns in diameter, with a coating of polymethylmethacrylate and carbon black, about 20 weight percent dispersed therein. Some sediment was noted, for example about 20 percent after about 5 days.

#### Preparation of Yellow Pigment Dispersion

##### 8% Solids Loading With 1:1 Ratio of Surfactant to Pigment

20.0 Grams of poly(ethylene glycol)- $\alpha$ -methyl ether- $\omega$ -methyl p-tert-octylphenyl phosphate hydrolyzable cleavable nonionic surfactant, 20.0 g (grams) Yellow 17 pigment and 460.0 grams of distilled water, were mixed in a Microfluidizer. To assess stability of the generated cyan pigment dispersion, two methods were used

- i) The dispersion was centrifuged at 4,000 rpm for 2 minutes and the weight of sediment measured.
- ii) The dispersion was retained, without agitation for 2 months, and the sediment measured.

#### Results

The pigment dispersion showed excellent stability, with no sediment measured from either of the above sedimentation methods.

#### Aggregation of Yellow Toner

260.0 Grams of the latex emulsion as prepared in Example I and 270.0 grams of a dilute aqueous yellow pigment dispersion containing 230.4 grams of the Yellow Pigment 17 dispersion prepared as above, 2.4 grams of cationic surfactant SANIZOL B™ and 37.2 grams of deionized water were simultaneously added to 350 milliliters of water with high shear stirring by means of a polytron. The resulting mixture was transferred to a 2 liter reaction vessel and heated at a temperature of 50° C. for 2.2 hours resulting in aggregates of a size of 5.6 microns and a GSD of 1.19 before 30 milliliters of 20 percent aqueous NEOGEN RTM solution was added. Subsequently, the mixture was heated to 93° C. and held there for a period of 3 hours before cooling down to room temperature, filtered, washed with water, and dried in a freeze dryer. The final toner product of 92 weight percent of the Example I polymer and 8 weight percent of Yellow Pigment 17 evidenced a particle size of 6.0 microns in volume average diameter with a particle size distribution

of 1.22 as measured on a Coulter Counter, and was shown to be smooth and spherical in shape by scanning electron microscopy. The toner exhibited a tribo charge of -44 and -21  $\mu$ C/gram at 20 and 80 percent relative humidity, respectively.

#### Comparative Aggregation of Yellow Toner

260.0 Grams of the latex emulsion as prepared in Example I and 220.0 grams of an aqueous yellow pigment dispersion containing 32 grams of Yellow Pigment 17 having a solids loading of 28.8 percent, and 2.4 grams of cationic surfactant SANIZOL BTM were simultaneously added to 400 milliliters of water with high shear stirring by means of a polytron. The resulting mixture was transferred to a 2 liter reaction vessel and heated at a temperature of 50° C. for 2.0 hours resulting in aggregates of a size of 5.8 microns and a GSD of 1.19 before 30 milliliters of 20 percent aqueous NEOGEN R™ solution was added. Subsequently, the mixture was heated to 93° C. and held there for a period of 3 hours before cooling down to room temperature, filtered, washed with water, and dried in a freeze dryer. The final toner product of 92 percent Example I polymer and 8 percent Yellow Pigment 17 evidenced a particle size of 6.4 microns in volume average diameter with a particle size distribution of 1.22 as measured on a Coulter Counter, and was shown to be smooth and spherical in shape by scanning electron microscopy. The toner exhibited a tribo charge of -38 and -17  $\mu$ C/gram at 20 and 80 percent relative humidity, respectively. Sedimentation was noted after about 3 days as measured by the above methods, reference the yellow toner preparation.

#### Preparation of Magenta Pigment Dispersion

##### 8% Solids Loading with 1:1 Ratio of Surfactant to Pigment

20.0 Grams of poly(ethylene glycol)- $\alpha$ -methyl ether- $\omega$ -methyl p-tert-octylphenyl phosphate hydrolyzable cleavable nonionic surfactant, 20.0 g R81:3 pigment and 460.0 g distilled water, were mixed in a Microfluidizer (Microfluidizer Corporation, Model Number M110-Y), at 15000 psi for 5 cycles.

To assess stability of the magenta pigment dispersion, two methods were used

- i) The dispersion was centrifuged at 4000 rpm for 2 minutes and the weight of sediment measured.
- ii) The dispersion was retained, without agitation for 2 months, and the sediment measured.

#### Results

The pigment dispersion showed excellent stability, that is it characteristics and the color did not change for one week, with no sediment measured from either of the above sedimentation methods.

#### Aggregation of Magenta Toner

260.0 Grams of the latex emulsion as prepared in Example I and a dilute dispersion of 168.0 grams of the aqueous magenta R81:3 pigment dispersion prepared as above, 2.4 grams of cationic surfactant SANIZOL BTM and 49.6 grams of deionized water were simultaneously added to 400 milliliters of water with high shear stirring by means of a polytron. The resulting mixture was transferred to a 2 liter reaction vessel and heated at a temperature of 50° C. for 2.0 hours resulting in aggregates of a size of 5.7 microns and GSD of 1.21 before 30 milliliters of 20 percent aqueous NEOGEN R™ solution were added. Subsequently, the mixture was heated to 93° C. and held there for a period of 3 hours before cooling down to room temperature, filtered, washed with water, and dried in a freeze dryer. The final toner product of 95 percent polymer and 5 percent Pigment Red 81:3 evidenced a particle size of 5.9 microns in volume average diameter with a particle size distribution of 1.21 as

measured on a Coulter Counter, and was shown to be of potato shape by scanning electron microscopy. The toner exhibited a tribo charge of -45 and -22  $\mu$ C/gram at 20 and 80 percent relative humidity, respectively.

5 Toner tribo was obtained by mixing in all instances the toner with carrier as indicated herein in Example I.

#### Comparative Aggregation of Magenta Toner

260.0 Grams of the latex emulsion as prepared in Example I and 220.0 grams of an aqueous magenta pigment dispersion containing 32 grams of Magenta Pigment R81:3 having a solids loading of 21 percent, and 2.4 grams of cationic surfactant SANIZOL BTM were simultaneously added to 400 milliliters of water with high shear stirring by means of a polytron. The resulting mixture was transferred to a 2 liter reaction vessel and heated at a temperature of 50° C. for 2.0 hours resulting in aggregates of a size of 5.9 microns and GSD of 1.20 before 30 milliliters of 20 percent aqueous NEOGEN R™ solution were added. Subsequently, the mixture was heated to 93° C. and held there for a period of 3 hours before cooling down to room temperature, filtered, washed with water, and dried in a freeze dryer. The final toner product of 95 percent polymer and 5 percent Pigment Red 81:3 evidenced a particle size of 6.0 microns in volume average diameter with a particle size distribution of 1.20 as measured on a Coulter Counter, and was shown to be of potato shape by scanning electron microscopy. The toner exhibited a tribo charge of -30 and -13  $\mu$ C/gram at 20 and 80 percent relative humidity, respectively. Some sedimentation was noted after about 7 days.

30 Toner tribo was obtained by mixing in all instances the toner with carrier as indicated herein in Example I.

#### Preparation of Black Pigment Dispersion

##### 7% Solids Loading with 1:1 Ratio of Surfactant to Pigment

17.5 Grams of poly(ethylene glycol)- $\alpha$ -methyl ether- $\omega$ -methyl p-tert-octylphenyl phosphate hydrolyzable cleavable nonionic surfactant, 17.5 grams of Black REGAL 330® pigment and 465 grams of distilled water, were mixed in a Microfluidizer (Microfluidizer Corporation, Model Number M110-Y), at 15,000 psi for 5 cycles.

35 To assess the stability of the above generated black pigment dispersion, two methods were used

- i) The dispersion was centrifuged at 4,000 rpm for 2 minutes and the weight of sediment measured.
- ii) The dispersion was retained, without agitation for 2 months, and the sediment measured.

#### Results

The above generated black pigment dispersion showed excellent stability, with no sediment was measured from either of the above sedimentation methods.

#### Aggregation of Black Toner

260.0 Grams of the latex emulsion as prepared in Example I and 220.0 grams of a dilute aqueous black pigment dispersion containing 192 grams of the carbon black REGAL 330® pigment dispersion prepared as above with 2.4 grams of cationic surfactant SANIZOL BTM and 25.6 grams of deionized water were simultaneously added to 400 milliliters of water with high shear stirring by means of a polytron. The resulting mixture was transferred to a 2 liter reaction vessel and heated at a temperature of 50° C. for 2.0 hours resulting in aggregates of a size of 6.0 microns and GSD of 1.21 before 30 milliliters of 20 percent aqueous NEOGEN R™ solution were added. Subsequently, the mixture was heated to 93° C. and held there for a period of 3 hours before cooling down to room temperature, filtered, washed with water, and dried in a freeze dryer. The final toner product of 95 percent polymer and 5 percent REGAL 330® carbon black pigment evidenced a particle size of 6.1

microns in volume average diameter with a particle size distribution of 1.22 as measured on a Coulter Counter, and was shown to be of potato shape by scanning electron microscopy. The toner exhibited a tribo charge of -40 and -19  $\mu$ C/gram at 20 and 80 percent relative humidity, respectively.

#### Comparative Aggregation of Black Toner

260.0 Grams of the latex emulsion as prepared in Example I and 220.0 grams of an aqueous black pigment dispersion containing 32 grams of carbon black REGAL 330® pigment having a solids loading of 21 percent, and 2.4 grams of cationic surfactant SANIZOL B™ were simultaneously added to 400 milliliters of water with high shear stirring by means of a polytron. The resulting mixture was transferred to a 2 liter reaction vessel and heated at a temperature of 50° C. for 2.0 hours resulting in aggregates of a size of 6.2 microns and GSD of 1.22 before 30 milliliters of 20 percent aqueous NEOGEN R™ solution were added. Subsequently, the mixture was heated to 93° C. and held there for a period of 3 hours before cooling down to room temperature, filtered, washed with water, and dried in a freeze dryer. The final toner product of 95 percent polymer and 5 percent REGAL 330® carbon black pigment evidenced a particle size of 6.6 microns in volume average diameter with a particle size distribution of 1.22 as measured on a Coulter Counter, and was shown to be of potato shape by scanning electron microscopy. The toner exhibited a tribo charge of -35 and -15  $\mu$ C/gram at 20 and 80 percent relative humidity, respectively.

Sediment was noted after 10 days.

#### Preparation of Surfactants

##### EXAMPLE I

Synthesis of Poly(ethylene glycol)Methyl 4-tert-octylphenyl Phosphate (XI) Wherein m is About 40

(XI)



#### Preparation of 4-tert-octylphenyl Dichlorophosphate

In a 500 milliliter round bottomed flask equipped with a magnetic stirrer and fitted with a reflux condenser, which was connected to a magnesium sulfate dry tube, were placed 25.0 grams (0.121 mole) of 4-tert-octylphenol, 57 grams (0.372 mole) of phosphorus oxychloride, and 0.35 gram (0.0036 mole) of magnesium chloride. The reaction mixture resulting was then heated to a reflux temperature of 110° C. and maintained at this temperature for 6 hours. The unreacted phosphorus oxychloride was distilled off and the reaction mixture was cooled to room temperature, about 25° C., to provide an oily mixture which contains 39.8 grams of 4-tert-octylphenyl dichlorophosphate.

In a 3 liter round bottomed flask equipped with a mechanical stirrer and fitted with an 100 milliliter addition funnel were added the 4-tert-octylphenyl dichlorophosphate as prepared above and 250 milliliters of anhydrous toluene, while in the addition funnel were placed 3.9 grams (0.121 mol) of methanol and 9.6 grams (0.121 mol) of pyridine. The flask was cooled with an ice bath and the mixture of methanol and pyridine was added through the addition funnel over a period of 0.5 hour. After the addition, the reaction mixture was stirred for an additional 1.0 hour. Into this mixture were added a solution of 182 grams of poly(ethylene glycol)

obtained from Aldrich Chemicals and with an average molecular weight  $M_w$  of 1,500, in 500 milliliters of anhydrous toluene and then followed by the addition of 9.6 grams of pyridine. After stirring for 0.5 hour, the ice bath was removed, and the reaction mixture was stirred for 12 hours. The precipitated pyridine hydrochloride solids were filtered off and the liquid mixture was concentrated by distilling the volatile materials to yield 195 grams of a waxy solid. The surfactant composition product (XI) was characterized by proton NMR. The chemical shifts in  $CDCl_3$  are: 0.7 (s), 1.36 (s), 1.72 (s), 3.66 (m, PEG backbone), 3.84 (d), 4.27 (m), 7.12 (d), 7.31 (d).

#### EXAMPLE II

Synthesis of Poly(ethylene glycol)  $\alpha$ -Methyl Ether  $\omega$ -Methyl 4-tert-octylphenyl Phosphate (XII) Wherein m is About 17:

(XII)



In a one liter round bottomed flask equipped with a magnetic stirrer and fitted with a reflux condenser, which condenser was connected to a magnesium sulfate dry tube, were placed 250 milliliters of anhydrous toluene and 100 grams of poly(ethylene glycol)monomethyl ether with an average molecular weight of 750. The flask was cooled with an ice bath, and to the stirred mixture there were added 45 grams (0.139 mol) of 4-tert-octylphenyl dichlorophosphate and 11 grams (0.139 mol) of pyridine. After 0.5 hour, the ice bath was removed and the reaction mixture was stirred at room temperature for 5.0 hours. The reaction was completed by adding 20 milliliters of methanol and 11.0 grams of pyridine, and the stirring was maintained for another 3.0 hours. The precipitated pyridine hydrochloride solids were removed by filtration, and the filtrate was concentrated under reduced pressure to yield 125 grams of a liquid. The surfactant composition product (XII) was characterized by proton NMR. The chemical shifts in  $CDCl_3$  are: 0.7 (s), 1.36 (s), 1.71 (s), 3.38 (s), 3.66 (m, PEG backbone), 3.85 (d), 4.27 (m), 7.12 (d), 7.34 (d).

#### EXAMPLE III

Synthesis of Bis[poly(ethylene glycol)]  $\alpha$ -Methyl Ether  $\omega$ -Methyl 4-tert-octylphenyl Phosphate (XIII) Wherein m is About 17

(XIII)



In a one liter round bottomed flask equipped with a magnetic stirrer and fitted with a reflux condenser, which was connected to a magnesium sulfate dry tube, were placed 150 milliliters of anhydrous toluene and 110 grams of poly(ethylene glycol)monomethyl ether with an average molecular weight of 750. The flask was cooled with an ice bath, and to the stirred mixture there were added 22.6 grams (0.07 mol) of 4-tert-octylphenyl dichlorophosphate and 11.0

grams (0.139 mol) of pyridine. After 0.5 hour, the ice bath was removed and the reaction mixture was stirred at room temperature for 5.0 hours. The precipitated pyridine hydrochloride solids were removed by filtration, and the liquid filtrate was concentrated under reduced pressure to yield 118 grams of a waxy solid. The surfactant composition product (XIII) was characterized by proton NMR. The chemical shifts in  $\text{CDCl}_3$  are: 0.7 (s), 1.36 (s), 1.70 (s), 3.39 (s), 3.66 (m, PEG backbone), 4.27 (m), 7.10 (d), 7.35 (d).

#### EXAMPLE IV

Synthesis of Bis[poly(ethylene glycol)]  $\alpha$ -Methyl Ether  $\omega$ -Methyl 4-Tert-octylphenyl Phosphate (XIII) Wherein M is About 40



In a 3 liter round bottomed flask equipped with a mechanical stirrer and fitted with an 100 milliliters addition funnel, were added the 4-tert-octylphenyl dichlorophosphate as prepared above and 250 milliliters of anhydrous toluene, while in the addition funnel were placed 3.9 grams (0.121 mol) of methanol and 9.6 grams (0.121 mol) of pyridine. The flask was cooled with an ice bath and the mixture of methanol and pyridine was added through the addition funnel over a period of 0.5 hour. After the addition, the reaction mixture was stirred for an additional 1.0 hour. Into this mixture was added a solution of 90 grams of poly(ethylene glycol) with an average molecular weight of 1,500 in 500 milliliters of anhydrous toluene and there followed by 20 grams of pyridine. After stirring for 0.5 hour, the ice bath was removed, and the reaction mixture was stirred for 12.0 hours. The precipitated pyridine hydrochloride solids were filtered off and the liquid mixture remaining was concentrated by distilling the volatile materials to yield 115 grams of a liquid. The surfactant composition product (XIV) was characterized by proton NMR. The chemical shifts in  $\text{CDCl}_3$  are: 0.71 (s), 1.37 (s), 1.72 (s), 3.67 (m, PEG backbone), 4.35 (d), 4.27 (m), 7.12 (d), 7.32 (d).

#### EXAMPLES V AND VI

Examples II and III were repeated substituting, respectively, a poly(ethylene glycol)monomethyl ether with an average molecular weight of 2,000 for the poly(ethylene glycol)monomethyl ether of Examples II and III. There were obtained nonionic surfactants (XV) and (XVI) whose structures are represented by Formulas (XII) and (XIII), wherein m is about 45, respectively. The chemical shifts of surfactant (XV) in  $\text{CDCl}_3$  are: 0.7 (s), 1.35 (s), 1.71 (s), 3.37 (s), 3.67 (m, PEG backbone), 3.84 (d), 4.27 (m), 7.12 (d), 7.33 (d). The chemical shifts of surfactant (XVI) in  $\text{CDCl}_3$  are: 0.69 (s), 1.36 (s), 1.70 (s), 3.40 (s), 3.66 (m, PEG backbone), 4.26 (m), 7.10 (d), 7.34 (d).

#### EXAMPLE VII

Example II was repeated substituting dodecylphenol for the 4-tert-octylphenol of Example II, resulting in the surfactant (XVII) wherein m is about 17

(XVII)



The chemical shifts of surfactant (XVII) in  $\text{CDCl}_3$  are: 0.85 (t), 1.30 (m), 2.51(t), 3.38 (s), 3.66 (m, PEG backbone), 3.85 (d), 4.27 (m), 7.10 (d), 7.34 (d).

Other modifications of the present invention may occur to those skilled in the art subsequent to a review of the present application and these modifications, including equivalents

(XIV)



thereof, are intended to be included within the scope of the present invention.

What is claimed is:

1. A process for the preparation of toner comprising mixing (1) a colorant dispersion containing a nonionic surfactant, and (2) a latex emulsion, and wherein the latex emulsion contains resin and a surfactant, and wherein the colorant nonionic surfactant is of the Formulas (I) or (II), or optionally mixtures thereof

(I)



(II)



wherein  $R^1$  is a hydrophobic aliphatic, or hydrophobic aromatic group;  $R^2$  is selected from the group consisting of hydrogen, alkyl, aryl, alkylaryl, and alkylaryalkyl;  $R^3$  is hydrogen or alkyl; A is a hydrophilic polymer chain, and m represents the number of A segments.

2. A process in accordance with claim 1 wherein  $R^1$  is a hydrophobic moiety of alkyl or aryl; and there is accomplished a heating below about or equal to about the resin latex glass transition temperature to form aggregates followed by heating above about or equal to about the resin glass transition temperature to coalesce the aggregates.

3. A process in accordance with claim 2 wherein  $R^1$  is alkyl, m is a number of from about 2 to about 60, and said hydrophilic polymer A is a poly(oxyalkylene glycol) selected from the group consisting of a branched polyoxyalkylene glycol, a block polyoxyalkylene glycol and a homopolymeric polyoxyalkylene glycol.

4. A process in accordance with claim 2 wherein m is a number of from about 5 to about 60, or from about 10 to about 50.

5. A process in accordance with claim 2 wherein the weight average molecular weight of A is from about 100 to about 3,000.

6. A process in accordance with claim 2 wherein R<sup>1</sup> is methylphenyl, ethylphenyl, propylphenyl, butylphenyl, pentylphenyl, hexylphenyl, octylphenyl, or nonylphenyl; R<sup>2</sup> is hydrogen, methyl, ethyl, methylphenyl, or propyl; R<sup>3</sup> is methyl, ethyl, propyl, or butyl; and A is polyoxyalkylene glycol, polyethylene glycol, or polypropylene glycol.

7. A process in accordance with claim 2 wherein R<sup>1</sup> is an alkylaryl group, or an alkylaryl group with a substituent of fluoride, chloride, or bromide, wherein alkyl contains from about 2 to about 30 carbon atoms; R<sup>2</sup> alkyl contains from 1 to about 30 carbon atoms; R<sup>3</sup> alkyl contains from 1 to about 3 carbon atoms; and wherein A is a hydrophilic poly (oxyalkylene glycol) selected from the group consisting of a branched, block or homopolymeric polyoxyalkylene glycol derived from alkylene oxides with from about 2 to about 4 carbon atoms.

8. A process in accordance with claim 2 wherein the latex resin is generated from the polymerization of monomers to provide a latex emulsion with submicron resin particles in the size range of from about 0.05 to about 0.3 micron in volume average diameter, and wherein the latex contains an ionic surfactant, a water soluble initiator and a chain transfer agent; adding anionic surfactant to substantially retain the size of the toner aggregates formed; thereafter coalescing or fusing said aggregates by heating; and optionally isolating, washing, and drying the toner.

9. A process in accordance with claim 8 wherein isolating, washing and drying are accomplished.

10. A process in accordance with claim 2 wherein R<sup>1</sup> is a an alkylaryl, or an alkylaryl group with a substituent of fluoride, chloride, or bromide, wherein alkyl contains from about 2 to about 30 carbon atoms; R<sup>2</sup> is an alkyl containing from about 1 to about 30 carbon atoms; R<sup>3</sup> is a hydrogen or an alkyl of from about 1 to about 3 carbon atoms, wherein A is a poly(ethylene glycol); and wherein the molecular weight M<sub>n</sub> of A is from about 104 to about 2,500.

11. A process in accordance with claim 2 wherein R<sup>2</sup> is an alkylphenyl with an alkyl of about 4 to about 30 carbon atoms, or wherein R<sup>2</sup> is an alkyl with from 1 to about 6 carbon atoms.

12. A process in accordance with claim 11 wherein said alkylphenyl is an octylphenyl, and R<sup>2</sup> is a methyl.

13. A process in accordance with claim 1 wherein R<sup>2</sup> is hydrogen or methyl, and wherein said poly(ethylene glycol) has a number of repeat units of from about 4 to about 50.

14. A process in accordance with claim 1 wherein said nonionic colorant surfactant is selected in an amount of from about 0.05 to about 60 weight percent based on the total weight of the colorant dispersion solids.

15. A process in accordance with claim 1 wherein said surfactant is cleavable, or hydrolyzable, and is selected in an amount of from about 1 to about 12 weight percent.

16. A process in accordance with claim 2 wherein the temperature at which said aggregation is accomplished controls the size of the aggregates, and wherein the final toner size is from about 2 to about 15 microns in volume average diameter.

17. A process in accordance with claim 16 wherein the aggregation temperature is from about 45° C. to about 55° C., and wherein the coalescence or fusion temperature is from about 85° C. to about 95° C.

18. A process in accordance with claim 1 wherein the colorant is a pigment and wherein said pigment dispersion contains an ionic surfactant, and the latex emulsion contains an ionic surfactant of opposite charge polarity to that of ionic surfactant present in said colorant dispersion.

19. A process in accordance with claim 2 wherein the aggregation is accomplished at a temperature of about 15° C. to about 1° C. below the Tg of the latex resin for a duration of from about 0.5 hour to about 3 hours; and wherein the coalescence or fusion of the components of aggregates for

the formation of integral toner particles comprised of colorant, and resin is accomplished at a temperature of from about 85° C. to about 95° C. for a duration of from about 1 hour to about 5 hours.

5 20. A process in accordance with claim 1 wherein the latex resin, or polymer is selected from the group consisting of poly(styrene-alkyl acrylate), poly(styrene-1,3-diene), poly(styrene-alkyl methacrylate), poly(styrene-alkyl acrylate-acrylic acid), poly(styrene-1,3-diene-acrylic acid), poly(styrene-alkyl methacrylate-acrylic acid), poly(alkyl methacrylate-alkyl acrylate), poly(aryl methacrylate-alkyl acrylate), poly(alkyl methacrylate-acrylic acid), poly(styrene-alkyl acrylate-acrylonitrile-acrylic acid), poly(styrene-1,3-diene-acrylonitrile-acrylic acid), and poly(alkyl acrylate-acrylonitrile-acrylic acid).

21. A process in accordance with claim 2 wherein the latex resin is selected from the group consisting of poly (styrene-butadiene), poly(methylstyrene-butadiene), poly (methyl methacrylate-butadiene), poly(ethyl methacrylate-butadiene), poly(propyl methacrylate-butadiene), poly(butyl methacrylate-butadiene), poly(methyl acrylate-butadiene), poly(ethyl acrylate-butadiene), poly(propyl acrylate-butadiene), poly(butyl acrylate-butadiene), poly(styrene-isoprene), poly(methylstyrene-isoprene), poly(methyl methacrylate-isoprene), poly(ethyl methacrylate-isoprene), poly(propyl methacrylate-isoprene), poly(butyl methacrylate-isoprene), poly(methyl acrylate-isoprene), poly(ethyl acrylate-isoprene), poly(propyl acrylate-isoprene), and poly(butyl acrylate-isoprene); poly(styrene-propyl acrylate), poly(styrene-butyl acrylate), poly(styrene-butadiene-acrylic acid), poly(styrene-butadiene-methacrylic acid), poly(styrene-butadiene-acrylonitrile-acrylic acid), poly(styrene-butyl acrylate-acrylic acid), poly(styrene-butyl acrylate-methacrylic acid), poly(styrene-butyl acrylate-acrylonitrile), and poly(styrene-butyl acrylate-acrylonitrile-acrylic acid); and wherein said colorant is a pigment, or a dye.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235



wherein R<sup>1</sup> is a hydrophobic group; R<sup>2</sup> is selected from the group consisting of hydrogen, alkyl, aryl, alkylaryl, and alkylarylalkyl; R<sup>3</sup> is hydrogen or alkyl; A is a hydrophilic segment; and m represents the number of A segments.

27. A process in accordance with claim 26 wherein said toner is isolated, washed and dried, and said toner is of a volume average diameter of from about 1 to about 20 microns.

28. A process in accordance with claim 1 wherein the colorant nonionic surfactant is selected from the group consisting of poly(ethylene glycol)methyl p-tert-octylphenyl phosphate, poly(ethylene glycol)- $\alpha$ -methyl ether- $\omega$ -methyl p-tert-octylphenyl phosphate, poly(ethylene glycol)methyl decylphenyl phosphate, poly(ethylene glycol)- $\alpha$ -methyl ether- $\omega$ -methyl dodecylphenyl phosphate, bis [poly(ethylene glycol)- $\alpha$ -methyl ether]- $\omega$ -p-tert-octylphenyl phosphate, poly(ethylene glycol)- $\alpha$ , $\omega$ -methyl p-tert-octylphenyl phosphate, poly(ethylene glycol)ethyl p-tert-octylphenyl phosphate, poly(ethylene glycol)- $\alpha$ -methyl ether- $\omega$ -ethyl p-tert-octylphenyl phosphate, poly(ethylene glycol)phenyl p-tert-octylphenyl phosphate, poly(ethylene glycol)- $\alpha$ -methyl ether- $\omega$ -phenyl p-tert-octylphenyl phosphate, poly(ethylene glycol)tolyl p-tert-octylphenyl phosphate, poly(ethylene glycol)- $\alpha$ -methyl ether- $\omega$ -tolyl p-tert-octylphenyl phosphate, and poly(ethylene oxide-co-propylene oxide)methyl p-tert-octylphenyl phosphate, wherein the polymer chain optionally contains from about 5 to about 50 repeating units or segments.

29. A process for the preparation of toner comprising mixing a colorant dispersion containing a surfactant with a latex emulsion, and wherein the colorant dispersion surfactant is represented by Formulas (I), (II) or (III); or optionally mixtures thereof



-continued

(I)

5



(II)

10

wherein R<sup>1</sup> is a hydrophobic moiety; R<sup>2</sup> is selected from the group consisting of hydrogen, alkyl and aryl; R<sup>3</sup> is hydrogen or alkyl; A is a hydrophilic polymer chain; and m is the number of repeating segments of the hydrophilic polymer chain A.

30. A process in accordance with claim 29 wherein said surfactant is nonionic.

31. A process in accordance with claim 29 wherein the surfactant is of Formula (I).

32. A process in accordance with claim 29 wherein the surfactant is of Formula (II).

33. A process in accordance with claim 29 wherein the surfactant is of Formula (III).

34. A process in accordance with claim 1 wherein said nonionic surfactant is of Formula (I).

35. A process in accordance with claim 1 wherein said nonionic surfactant is of Formula (II).

36. A process in accordance with claim 1 wherein said nonionic surfactant is of Formula (III).

37. A process for the stabilization of a colorant dispersion which comprises mixing a colorant and a surfactant represented by Formulas (I), (II) or (III); or optionally mixtures thereof

35



55

wherein R<sup>1</sup> is a hydrophobic group; R<sup>2</sup> is hydrogen, aliphatic, or aromatic; A is a hydrophilic chain; and m represent the number of repeating segments.

38. A process in accordance with claim 1 wherein said A is polyethylene glycol and said m is a number of about 17.

39. A toner obtained by the process of claim 1.

40. A process in accordance with claim 1 wherein said nonionic surfactant is poly(ethylene glycol)- $\alpha$ -methyl ether- $\omega$ -methyl p-tert-octylphenyl.

41. A process in accordance with claim 1 wherein said nonionic surfactant is of the formula

31



wherein m is about 17.

42. A process in accordance with claim 1 wherein said nonionic surfactant is of the formula



wherein m is about 40.

43. A process in accordance with claim 1 wherein said nonionic surfactant is of the formula



wherein m is about 40.

44. A process for the preparation of toner consisting essentially of mixing (1) a colorant dispersion containing a nonionic surfactant, and (2) a latex emulsion, and wherein

the latex emulsion contains resin and a surfactant, and wherein the colorant nonionic surfactant is of the Formulas (I) or (II), or optionally mixtures thereof



wherein R<sup>1</sup> is a hydrophobic aliphatic, or hydrophobic aromatic group; R<sup>2</sup> is selected from the group consisting of hydrogen, alkyl, aryl, alkylaryl, and alkylarylalkyl; R<sup>3</sup> is

hydrogen or alkyl; A is a hydrophilic polymer chain, and m represents the number of A segments.

\* \* \* \* \*

40

45

50

55

60

65